# EUROPEAN PATENT SPECIFICATION

(11) **EP 1 356 142 B1**
(45) Date of publication and mention of the grant of the patent: **19.04.2006**
(21) Application number: 01991772.3
(22) Date of filing: 04.12.2001
(51) Int. Cl.: D01F 6/06, D01F 6/46, D01F 1/10

(54) **NON-POSTDRAWN POLYOLEFIN FIBERS WITH HIGH TENACITY**
NICHT NACHVERSTRECKTE POLYOLEFINFASERN HOHER FESTIGKEIT
FIBRES DE POLYOLEFINES NON PRE-ETIREE A HAUTE TENACITE

(30) Priority: 07.12.2000 EP 00126834
(43) Date of publication of application: 29.10.2003
(73) Proprietor: Borealis GmbH, 2323 Schwechat-Mannswörth (AT)
(72) Inventor: VERPOEST, Marijke, B-9520 Sint-Lievens-Houtem (BE); ROHNE, Gunhild, N-2819 Gjovik (NO); GAHLEITNER, Markus, A-4501 Neuhofen/Krems (AT)
(74) Representative: VA TECH Patente GmbH & Co
(86) International application number: PCT/EP2001/014155
(87) International publication number: WO 2002/046502

(56) References cited:
- EP-A- 0 569 860
- EP-A- 0 790 262
- EP-A- 0 854 155
- EP-A- 0 878 567
- WO-A-99/24478
- WO-A-99/24479
- US-A- 5 137 973

## Description

The invention relates to non-postdrawn polyolefin fibers with high tenacity from propylene polymers as well as to a process for producing them.

Fibers from propylene polymers are known (Ullmann's Encyclopedia of Industrial Chemistry, Vol. A10, p. 536-542, Weinheim 1987).

Known methods for producing high tenacity fibers are oxidative chain scission degradation of hot spun fibers in conjunction with a delayed quench step (U.S. 5 281 378, US 5 318 735), the use of reactor-grade propylene polymers produced by single-site catalysis (EP 0 854 212) for producing the fibers, or the use of blends consisting of mixtures of propylene homopolymers, propylene copolymers and heterophasic propylene polymers being stabilized with organic phosphites, phenolic antioxidants or HALS-compounds for producing the fibers (EP 0 632 147). The disadvantage of these methods is, that non-postdrawn propylene polymer fibers having tenacity values of 2,0 to 5,0 cN/dtex cannot be realised.
EP 0 878 567 discloses non post-drawn polyolefin fibers having high tenacities and tensile elongations without specifying isotacticity and crystallinity of the used polypropylenes. The optional addition of nucleating agents is predicted to result in a decrease of the fiber's tenacity.
EP 0 569 860 discloses spunbond webs and nonwoven fabric laminates thereof made from polypropylene compositions having a MFI greater than 12 and comprising 0.1 t 0.3 wt% of a nucleating agent. Isotacticity and crystallinity of the used polypropylenes are not specified. The use of nucleating agents does not increase the fiber tenacity but improves the bonding strength of fabric laminates formed

It is the object of the present invention to provide non-postdrawn polyolefin fibers having tenacity values of 2,0 to 5,0 cN/dtex comprising propylene polymers.

According to the present invention, this object is achieved by non-postdrawn polyolefin fibers with high tenacity values of 2,0 to 5,0 cN/dtex, consisting essentially of predominantly isotactic propylene polymers having a crystallisation temperature of > 116 °C (DSC) and 0,001 to 2 % by weight, based on the propylene polymers used, of α-nucleating agents which are selected from the group consisting of
polymers which are different from isotactic propylene polymers, which are selected from the group consisting of
tetrafluoroethylene polymers, polycarbonates, polybutyleneterephthalate, polyethyleneterephthalate, 3-methylbutene polymers, 4-methylpentene-1-polymers, syndiotactic propylene polymers, polyphenyleneoxides, propylene-methylbutene copolymers, styrene-acrylonitrile copolymers, polyallyltrimethylsilanes and hydrolysed ethylene vinylacetate copoiymers,
and benzoic acid, benzoic acid derivatives, dibenzylidene sorbitol, derivatives of sorbitol, diphenylglycine, salts of C₆-C₁₈ aliphatic carboxylic acids, salts of C₇-C₁₃ aromatic carboxylic acids, phosphoric acid derivatives, talc and mixtures thereof.

The predominantly isotactic propylene polymers are essentially consisting of
(a) 50 - 100 wt% propylene polymers produced using Ziegler-Natta catalysts or metallocene catalysts, preferably propylene homopolymers and/or copolymers of propylene, ethylene and/or α-olefins with 4 to 18 carbon atoms and a propylene content of 80.0 to 99.9 % by weight in the form of random copolymers, block copolymers and/or random block copolymers, with melt indexes of 0.5 to 40 g/10 min at 230 °C/2.16 kg and preferably of 1 to 5 g/10 min at 230 °C/2.16 kg,
(b) 0 - 50 wt % of a polyolefin mixture with an Mw/Mn ratio of 2 to 6 and a melt index of 0,5 to 40 g/10 min at 230 °C/2.16 kg, essentially consisting of
   (b1) 60 to 98 % by weight of a crystalline copolymer of 85 to 95 % by weight of propylene and 15 to 0.5 % by weight of ethylene and/or an α-olefin of the general formula CH₂ = CHR, wherein R is a linear or branched alkyl group with 2 to 8 carbon atoms,
   (b2) 2 to 40 % by weight of an elastic copolymer of 20 to 70 % by weight of ethylene and 80 to 30 % by weight of propylene and/or an α-olefin of the general formula CH₂CHR, wherein R is a linear or branched alkyl group with 2 to 8 carbon atoms,
(c) 0 - 30 wt% of highly amorphous polypropylenes or propylene copolymers with a crystalline polypropylene or crystalline propylene copolymer content of less than 10 % by weight, an enthalpy of melting of less than 40 J/g and a melt index of 0.5 to 40 g/10 min at 230 °C/2.16 kg, the largely amorphous polypropylene being a homopolymer of propylene and/or a copolymer of propylene of at least 80 mole percent propylene and not more than 20 mol percent of one or more α-olefins of the general formula CH₂CHR, wherein R is a linear or branched alkyl group with 2 to 8 carbon atoms,
(d) 0 - 10 wt% of non-isotactic propylene homopolymers with a melting point of 145° to 165 °C, a melt viscosity of 200 Pa·s (200,000 cps) at 190 °C and a heat of crystallization of 4 to 10 calories per gram, 35 to 55 % by weight being soluble in diethyl ether,
(e) 0 - 30 wt% of modified propylene homopolymers and/or propylene copolymers with melt indexes of 0.5 to 40 g/10 min at 230 °C/2.16 kg and preferably of 2 to 5 g/10 min at 230 °C/2.16 kg, and a ratio of the intrinsic viscosity of the modified propylene polymer to the intrinsic viscosity of the basic unmodified polymer (component a) with largely the same weight average molecular weight of 0,2 to 0,95.

The polyolefin mixtures b) of crystalline copolymers and elastic copoiymers, optionaiiy contained in the non-postdrawn polyolefin fibers, are polymer mixtures described, for example, in the European patents 0 400 333 or 0 472 946.

The largely amorphous polypropylenes or propylene copolymers c), optionally contained in the non-postdrawn polyolefin fibers are, in particular, stereo block polypropylenes, which are prepared, for example, by using highly active Ziegler-Natta catalysts fixed on a metal oxide (Collette, J., Macromolecules 22 (1989), 3851 - 3858; German patent 28 30 160) or soluble Ziegler-Natta catalysts (de Candia, F., Makromol. Chem. 189 (1988), 815 - 821), optionally with subsequent reactive modification (European patent 636863) and/or degradation (European patent 640 850).

Examples for the non-isotactic propylene homopolymers d), optionally contained in the non-postdrawn polyolefin fibers are the products described p.e. in the European patent 0 475 307 or in the European patent 0 475 308.

The modified propylene polymers e), optionally contained in the non-postdrawn polyolefin fibers, can be produced by any number of processes, e.g. by treatment of the unmodified propylene polymer with thermal decomposing radical-forming agents and/or by treatment with ionizing radiation, where both treatments may optionally be accompanied or followed by a treatment with bi- or multifunctionally unsaturated monomers, e.g. butadiene, isoprene, dimethylbutadiene or divinylbenzene. Further processes may be suitable for the production of the modified propylene polymer, provided that the resulting modified propylene polymer meets the characteristics given above.

Examples for said modified propylene polymers e) optionally contained in the non-postdrawn polyolefin fibers, are, in particular:
- polypropylenes modified by the reaction of polypropylenes with bismaleimido compounds in the melt (EP-A-0 574 801; EP-A-0 574 804),
- polypropylenes modified by the treatment of polypropylenes with ionizing radiation in the solid phase (EP-A-0 190 889; EP-A-0 634 454),
- polypropylenes modified by the treatment of polypropylenes with peroxides in the solid phase (EP-A-0-384 431) or in the melt (EP-A-0-142724),
- polypropylenes modified by the treatment of polypropylenes with multifunctional, ethylenically unsaturated monomers using ionizing radiation (EP-A-0 678 527)
- polypropylenes modified by the treatment of poiypropylenes with multifunctional, ethylenically unsaturated monomers in the presence of peroxides in the melt (EP-A-0 688 817; EP-A-0 450 342)

These modified polypropylenes have melt indexes of 0.5 to 40 g/10 min at 230 °C/2.16 kg and preferably of 2 to 5 g/10 min at 230 °C/2.16 kg, and a ratio of the intrinsic viscosity of the modified propylene polymer to the intrinsic viscosity of the basic unmodified polymer (component a) with largely the same weight average molecular weight of 0,2 to 0,95.
These modified poylpropylene polymers normally exhibit strain hardening behaviour as usually defined in the literature.

Examples for tetrafluoroethylene polymers, optionally contained in the non-postdrawn poly-olefin fibers, are polytetrafluoroethylene, tetrafluoroethylene propylene copolymers and tetrafluoroethylene isobutylene copolymers.

Examples for polycarbonates, optionally contained in the non-postdrawn polyolefin fibers, are poly(4,4'-isopropylidenediphenylene carbonate) and copolycondensates based on 4,4'-isopropylidenebisphenol, 4,4'-tetrabromoisopropylidenebisphenol and/or 4,4'-hexabromoiso-propylidenebisphenol.

Examples for 3-methylbutene polymers, optionally contained in the non-postdrawn polyolefin fibers, are poly-3-methylbutene, 3-methylbutene 1-butene copolymers or 3-methylbutene isobutylene copolymers.

Examples for 4-methylpentene-1-polymers, optionally contained in the non-postdrawn poly-olefin fibers, are poly-4-methylpentene-1, 4-methylpentene-1 styrene copolymers or 4-methylpentene-1 propylene copolymers.

Examples for polyphenyleneoxides, optionally contained in the non-postdrawn polyolefin fibers, are poly-2,6-dimethylphenyleneoxide, poly-2,6-diisopropylphenyleneoxide or poly-2,6-diphenylphenyleneoxide.

Examples for C₇-C₁₃ benzoic acid derivatives, optionally contained in the non-postdrawn polyolefin fibers, are benzoic anhydride, o-toluic acid and 2,6-dimethylbenzoic acid.

Examples for sorbitol derivatives, optionally contained in the non-postdrawn polyolefin fibers, are di-(p-methylbenzylidene) sorbitol, trinaphthylidenesorbitol and naphthylmethylenesorbitol.

Examples for salts of C₇-C₁₃ aromatic carboxylic acids are sodium benzoate and tertiary-butylbenzoic acid aluminium salt.
A preferred aromatic carboxylic acid is sodium benzoate.

Examples for phosphoric acid derivatives are ammonium polyphosphate, cyclic calcium phosphate compounds, sodium-2,2'-methylenebis-(4,6-di-tert.-butylphenyl)phosphate and bis-(tertiary-butyl) phos-phoric acid sodium salt.

A preferred cyclic calcium phosphate compound, optionally contained in the non-postdrawn polyolefin fibers, is bis(2,6-di-tert.butyl-1-hydroxy)methane calcium phosphate.
A further α-nucleation method, which is also suitable, is a special reactor technique, where the catalyst is prepolymerised with monomers like vinylcyclohexane (VCH). This method is described in greater detail in e.g. EP 0 316 187 A2.
In addition to the nucleating agents mentioned above, the use of long-chain branched polypropylene with high melt strength for nucleation purposes as outlined e.g. in US 6,077,907 is included.

Preferred auxiliary materials are 0.01 to 2.5 % by weight of stabilizers and/or 0.01 to 1 % by weight of processing aids and/or, optionally, 0. 1 to 1 % by weight of antistatic agents and/or 0.2 to 3 % by weight of pigments and/or 2 to 20 % by weight of flame retardants, in each case based on the sum of the polypropylenes.

The stabilizers, contained in the inventive non-postdrawn polyolefin fibers, preferably are mixtures of 0.01 % to 0.6 % by weight of phenolic antioxidants, 0.01 % to 0.6 % by weight of 3-arylbenzofuranones, 0.01 % to 0.6 % by weight of processing stabilizers based on phosphites, 0.01 % to 0.6 % by weight of high temperature stabilizers based on disulfides and thioethers and/or 0.01 % to 0.8 % by weight of sterically hindered amines (HALS).

Suitable phenolic antioxidants are 2-t-butyl-4,6-dimethylphenol, 2,6-di-t-butyl-4-methylphenol, 2,6-di-t-butyl-4-isoamylphenol, 2,6-di-t-butyl-4-ethylphenol, 2-t-butyl-4,6-diisopropylphenol, 2,6-dicyclopentyl-4-methylphenol, 2,6-di-t-butyl-4-methoxymethylphenol, 2-t-butyl-4,6-dioctadecylphenol, 2,5-di-t-butylhydroquinone, 2,6-di-t-butyl-4,4-hexadecyloxyphe-nol, 2,2'-methylene-bis(6-t-butyl-4-methylphenol), 4,4'-thio-bis-(6-t-butyl-2-methylphenol), octade-cyl 3(3,5-di-t-butyl-4-hydroxyphenyl) propionate, 1,3,5-trimethyl-2,4,6-tris(3',5'-di-t-bu-tyl-4-hydroxybenzyl)benzene and/or pentaerythritol-tetrakis-3-(3,5-dit-butyl-4-hydroxyphenyl)-propionate.

As benzofuranone derivative, 5,7-di-t-butyl-3-(3,4-dimethylphenyl)-3H-benzofuran-2-one, in particular, is suitable.

As HALS compounds, bis-2,2,6,6-tetramethyl-4-piperidyl sebacate and/or poly-1,1,3,3-tetra-methylbutyl)-imino)-1,3,5-triazine-2,4-diyl)(2,2,6,6-tetramethylpiperidyl)-amino)-hexamethyle-ne-4-(2,2,6,6-tetramethyl)piperidyl)-imino) are particularly suitable.

As processing aids, the inventive non-postdrawn polyolefin fibers may contain calcium stearate, magnesium stearate and/or waxes.

Preferably, the fibres comprise conventional additives.

According to an advantageous embodiment of the present invention the predominantly isotactic propylene polymers comprise from 5 - 100 ppm of particles of inorganic oxides having a particle diameter from 0.05 - 10 *µ*m.

Inorganic oxides selected from the group consisting of ZnO, SnO, MgO, Al₂O₃, SiO₂, TiO₂, ZrO₂, HfO₂ and mixtures thereof in amounts of from 20 -40 ppm are preferred.
Still more preferred are particles of inorganic oxides of Al₂O₃ and/or SiO₂ and/or MgO having a particle diameter from 0.5 to 2.0 *µ*m.

A still further object of the present invention is a process for preparing the inventive non-postdrawn polyolefin fibers having tenacity values of 2,0 to 5,0 cN/dtex , characterized by melting of predominantly isotactic propylene polymers having a crystallisation temperature of > 116 °C (DSC) and 0,001 to 2 % by weight, based on the propylene polymers used, of α-nucleating agents which are selected from the group consisting of
polymers which are different from isotactic propylene polymers, which are selected from the group consisting of
tetrafluoroethylene polymers, polycarbonates, polybutyleneterephthalate, polyethyleneterephthalate, 3-methylbutene polymers, 4-methylpentene-1-polymers, syndiotactic propylene polymers, polyphenyleneoxides, propylene-methylbutene copolymers, styrene-acrylonitrile copolymers, polyallyltrimethylsilanes and hydrolysed ethylene vinylacetate copolymers,
and benzoic acid, benzoic acid derivatives, dibenzylidene sorbitol, derivatives of sorbitol, diphenylglycine, salts of C₆-C₁₈ aliphatic carbonic acids, salts of C₇-C₁₃ aromatic carbonic acids, phosphoric acid derivatives, talc
and mixtures thereof,
at temperatures of 220 to 325 °C, conveying the melt to spinnerets, extruding the melt into fibers and subsequently cooling the fibers and taking up the hot spun fibers at speeds of 1000 - 6000 m/min..

As plasticising extruder for melting the mixtures, especially single screw extruders or twin screw extruders with screw length of 28 to 30 D, preferably with flange-mounted static or dynamic mixers, are suitable. Sheer speeds can be adjusted to values of 10² /sec to 10³/sec by controlling the temperature and the rpm.

For uniformly metering the mixtures, which has been melted in the plasticizing extruder, over the melt distributor to the capillary die, melt pumps, preferably heated with biphenyl, are used for the melts, heated to 240° to 310 °C.

According to a feature of the present invention, the hot spun fibers are taken up by high speed galettes, cabling the fibers into multifilament yarns and winding up the non-postdrawn polyolefin fibers-containing yarns.

Preferred applications of the non-postdrawn polyolefin fibers are the manufacturing of nonwovens, preferred spunbond, carded or air bonded nonwovens; textile applications, carpets.

### Examples

For the production of polyolefin fibers, which are not drawn subsequently, the inventive method is explained, by way of example, by a method outlined in Fig. 1. In Fig. 1, 1 is the extruder, 2 the extrusion pump, 3 the spinneret, 4 the blast shaft, 5 the pull-off equipment and 6 the winder.

As extruder (1) for melting the polyolefin mixtures, a single screw extruder is used with a high homogenizing effect with a screw length of 34 D and a flange-mounted static mixer. The spinneret (3) has an internal diameter of 0.5 mm. In the pull-off equipment (5), the pulling-off can be accomplished directly by means of the winder (6). Possible pull-off speeds are 1000 to 6000 m/min.

The melt indices for propylene polymers were measured with a load of 2.16 kg at 230 °C. The melt index is that quantity of polymer in grams which the test apparatus standardized to DIN 53 735 extrudes within 10 minutes at a temperature of 230 °C under a weight of 2.16 kg.

Tenacity and tensile elongation are both determined according to DIN 53834/1.

### Example 1

For producing a polyolefin polymer blend for high speed melt spinning, a dry mixture consisting of 85 % by weight of a metallocene propylene homopolymer (melt index of 6.2 g/10 minutes at 230 °C/2.16 kg), 13 % by weight of a propylene ethylene copolymer (melt index of 4,2 g/10 minutes at 230 °C/2.16 kg, ethylene content 4,8 % by weight), 2 % by weight of a 4-methylpentene-1 propylene copolymer (melt index of 0,25 g/10 minutes at 230 °C/5 kg, propylene content 6,8 % by weight), and as adjuvants, the percentages in each case based on the sum of the propylene polymers, 0.25 % by weight of 2-t-butyl-4,6-diisopropylphenol, 0.2 % by weight of bis-2,2,6,6-tetramethyl-4-piperidyl sebacate and 0.2 % by weight of calcium stearate, is melt blended at a melt temperature of 230 °C In a twin screw extruder and granulated.

In the spinning equipment of Figure 1, the blend is melted in the extruder at a mass temperature of 275 °C. The melt is transferred by the extrusion pump to the spinneret and, at a spinneret temperature of 290 °C, drawn off through the blast shaft, which is cooled with compressed air at a temperature of 20 °C, and wound up at a speed of 4000 m/min.

The resulting polypropylene fiber, which is not postdrawn, has a tenacity of 3.6 cN/dtex and a tensile elongation of 105 %.

### Example 2

For producing a polyolefin polymer blend for high speed melt spinning, a dry mixture consisting of 90 % by weight of a metallocene propylene homopolymer (melt index of 6.2 g/10 minutes at 230 °C/2.16 kg), 5 % by weight of a random heterophasic propylene ethylene blockcopolymer (melt index of 8 g/10 minutes at 230 °C/2.16 kg, ethylene content 33 mol%) 5 % by weight of a propylene ethylene copolymer (melt index of 4,2 g/10 minutes at 230 °C/2.16 kg, ethylene content 4,8 % by weight) and, the percentages in each case based on the sum of the propylene polymers, 0,2 % by weight of dibenzylidene sorbitol, 0.25 % by weight of 3(3,5-di-t-butyl-4-hydroxyphenyl)proplonate, 0.2 % by weight of bis-2,2,6,6-tetra-methyl-4-piperidyl sebacate and 0.2 % by weight of magnesium stearate, is melt blended at a melt temperature of 220 °C in a twin screw extruder and granulated.

In the spinning equipment of Figure 1, the blend is melted in the extruder at a mass temperatureof 280 °C. The melt is transferred by the extrusion pump to the spinneret and, at a spinneret temperature of 285 °C, drawn off through the blast shaft, which is cooled with compressed air at a temperature of 20 °C, and wound up at a speed of 3500 m/min.

The resulting polypropylene fiber, which is not postdrawn, has a tenacity of 3.2 cN/dtex and a tensile elongation of 122 %.

### Example 3

For producing a polyolefin polymer blend for high speed melt spinning, a dry mixture consisting of 85 % by weight of a metallocene propylene homopolymer (melt index of 6.2 g/10 minutes at 230 °C/2.16 kg), 5 % of a propylene homopolymer having strain hardening behavior (melt index of 3,5 g/10 minutes at 230 °C/2.16 kg, strain hardening behaviour as usually defined in the literature), 10 % by weight of a Ziegler-Natta propylene homopolymer with high stereospecifity (melt index of 2,5 g/10 minutes at 230 °C/2.16 kg), and, the percentages in each case based on the sum of the propylene polymers, 0,35 % by weight of sodium-2,2'-methylenebis-(4,6-di-tert.-butylphenyl)phosphate, 0.25 % by weight of 2-t-butyl-4,6-diisopropylphenol, 0.2 % by weight of bis-2,2,6,6-tetramethyl-4-plperidyl seba-cate and 0.2 % by weight of calcium stearate, is melt blended at a melt temperature of 225 °C in a twin screw extruder and granulated.

In the spinning equipment of Figure 1, the blend is melted in the extruder at a mass temperature of 285 °C. The melt is transferred by the extrusion pump to the spinneret and, at a spinneret temperature of 290 °C, drawn off through the blast shaft, which is cooled with compressed air at a temperature of 20 °C, and wound up at a speed of 3000 m/min.

The resulting polypropylene fiber, which is not postdrawn, has a tenacity of 3.0 cN/dtex and a tensile elongation of 137 %.

## Claims

1. Non-postdrawn polyolefin fibers with high tenacity values of 2,0 to 5,0 cN/dtex, consisting essentially of predominantly isotactic propylene polymers having a crystallisation temperature of > 116 °C (DSC) and 0,001 to 2 % by weight, based on the propylene polymers used, of α-nucleating agents which are selected from the group consisting of
polymers which are different from isotactic propylene polymers, which are selected from the group consisting of
tetrafluoroethylene polymers, polycarbonates, polybutyleneterephthalate, polyethyleneterephthalate, 3-methylbutene polymers, 4-methylpentene-1-polymers, syndiotactic propylene polymers, polyphenyleneoxides, propylene-methylbutene copolymers, styrene-acrylonitrile copolymers, polyallyltrimethylsilanes and hydrolysed ethylene vinylacetate copolymers,
and benzoic acid, benzoic acid derivatives, dibenzylidene sorbitol, derivatives of sorbitol, diphenylglycine, salts of C₆-C₁₈ aliphatic carboxylic acids, salts of C₇-C₁₃ aromatic carboxylic acids, phosphoric acid derivatives, talc
and mixtures thereof.

2. Non-postdrawn polyolefin fibers as claimed in claim 1, wherein said predominantly isotactic propylene polymers are essentially consisting of
(a) 50 - 100 wt% propylene polymers produced using Ziegler-Natta catalysts or metallocene catalysts, preferably propylene homopolymers and/or copolymers of propylene, ethylene and/or α-olefins with 4 to 18 carbon atoms and a propylene content of 80.0 to 99.9 % by weight in the form of random copolymers, block copolymers and/or random block copolymers, with melt indexes of 0.5 to 40 g/10 min at 230 °C/2.16 kg.
(b) 0 - 50 wt % of a polyolefin mixture with an Mw/Mn ratio of 2 to 6 and a melt index of 0,5 to 40 g/10 min at 230 °C/2.16 kg, essentially consisting of
(b1) 60 to 98 % by weight of a crystalline copolymer of 85 to 95 % by weight of propylene and 15 to 0.5 % by weight of ethylene and/or an α-olefin of the general formula CH₂ = CHR, wherein R is a linear or branched alkyl group with 2 to 8 carbon atoms,
(b2) 2 to 40 % by weight of an elastic copolymer of 20 to 70 % by weight of ethylene and 80 to 30 % by weight of propylene and/or an α-olefin of the general formula CH₂CHR, wherein R is a linear or branched alkyl group with 2 to 8 carbon atoms,
(c) 0 - 30 wt% of highly amorphous polypropylenes or propylene copolymers with a crystalline polypropylene or crystalline propylene copolymer content of less than 10 % by weight, an enthalpy of melting of less than 40 J/g and a melt index of 0.5 to 40 g/10 min at 230 °C/2.16 kg, the largely amorphous polypropylene being a homopolymer of propylene and/or a copolymer of propylene of at least 80 mole percent propylene and not more than 20 mol percent of one or more α-olefins of the general formula CH₂CHR, wherein R is a linear or branched alkyl group with 2 to 8 carbon atoms,
(d) 0 - 10 wt% of non-isotactic propylene homopolymers with a melting point of 145° to 165 °C, a melt viscosity of 200 Pa·s (200,000 cps) at 190 °C and a heat of crystallization of 4 to 10 calories per gram, 35 to 55 % by weight being soluble in diethyl ether,
(e) 0 - 30 wt% of modified propylene homopolymers and/or propylene copolymers with melt indexes of 0.5 to 40 g/10 min at 230 °C/2.16 kg, and a ratio of the intrinsic viscosity of the modified propylene polymer to the intrinsic viscosity of the basic unmodified polymer (component a) with largely the same weight average molecular weight of 0,2 to 0,95.

3. Non-postdrawn polyolefin fibers as claimed in claim 1 or 2, further comprising conventional additives.

4. Non postdrawn polyolefin fibers as claimed in claim 3, wherein said conventional additives are 0.01 to 2.5 % by weight of stabilizers, 0.01 to 1 % by weight of processing aids and, optionally, 0.1 to 1 % by weight of antistatic agents, 0.2 to 3 % by weight of pigments and 2 to 20 % by weight of flame retardants, in each case based on the sum of the polypropylenes.

5. Non-postdrawn polyolefin fibers according to any one of claims 1 to 4 **characterized in that** the predominantly isotactic propylene polymers comprise from 5 - 100 ppm of particles of inorganic oxides having a particle diameter from 0.05 - 10 *µ*m.

6. Non-postdrawn polyolefin fibers according to claim 5, **characterized in that** the predominantly isotactic propylene polymers comprise from 20 -40 ppm of inorganic particles selected from the group consisting of ZnO, SnO, MgO, Al₂O₃, SiO₂, TiO₂, ZrO₂, HfO₂ and mixtures thereof.

7. Non-postdrawn polyolefin fibers according to one of claims 5 or 6, **characterized in that** the particles of inorganic oxides are Al₂O₃ and/or SiO₂ and/or MgO having a particle diameter from 0.5 to 2.0 *µ*m.

8. Process for preparing non-postdrawn polyolefin fibers according to any one of claims 1 to 7 , **characterised by** melting of predominantly isotactic propylene polymers according to any one of claims 1 - 7 and 0,001 to 2 % by weight, based on the propylene polymers used of α-nucleating agents according to claim 1 at temperatures of 220 to 325 °C, conveying the melt to spinnerets, extruding the melt into fibers and subsequently cooling the fibers and taking up the hot spun fibers at speeds of 1000 - 6000 m/min.

9. Process for preparing non-postdrawn polyolefin fibers as claimed in claim 8, **characterised in that** the hot spun fiber is taken up by high speed galettes, the fibers are cabled into multifilament yarns and the yarns containing the non-postdrawn polyolefin fibers are wound up.

10. Use of non-postdrawn polyolefin fibers of any one of the claims 1 to 7 for manufacturing of nonwovens for textile applications, and carpets.

11. Non-postdrawn polyolefin fibers as claimed in claim 2, wherein the propylene polymers according to 2 (a) have melt indexes of 1 to 5 g/10 min at 230 °C/2.16 kg.

12. Non-postdrawn polyolefin fibers as claimed in claim 2, wherein the modified propylene homopolymers and/or propylene copolymers according to 2 (e) have melt indexes of 2 to 5 g/10 min at 230°C/2.16 kg.

13. Use of non-postdrawn polyolefin fibers according to claim 10, **characterized in that** the nonwovens are spunbond, carded or air bonded nonwovens.

## Patentansprüche

1. Nichtnachverstreckte Polyolefinfasern mit hohen Feinheitsfestigkeitswerten von 2,0 bis 5,0 cN/dtex, im wesentlichen bestehend aus überwiegend isotaktischen Propylenpolymeren mit einer Kristallisationstemperatur von >116°C (DSC) und 0,001 bis 2 Gew.-%, bezogen auf die eingesetzten Propylenpolymere, an α-Nukleierungsmitteln, ausgewählt aus der Gruppe bestehend aus
von isotaktischen Propylenpolymeren verschiedenen Polymeren, ausgewählt aus der Gruppe, bestehend aus
Tetrafluorethylenpolymeren, Polycarbonaten, Polybutylenterephthalat, Polyethylenterephthalat, 3-Methylbutenpolymeren, 4-Methylpenten-1-polymeren, syndiotaktischen Propylenpolymeren, Polyphenylenoxiden, Propylenmethylbutencopolymeren,
Styrolacrylnitrilcopolymeren, Polyallyltrimethylsilanen und hydrolysierten Ethylenvinylacetatcopolymeren,
und Benzoesäure, Benzoesäurederivaten, Dibenzylidensorbit, Derivaten des Sorbits, Diphenylglycin, Salzen von C₆-C₁₈-aliphatischen Carbonsäuren, Salzen von C₇-C₁₃-aromatischen Carbonsäuren, Phosphorsäurederivaten, Talk und deren Mischungen.

2. Nichtnachverstreckte Polyolefinfasern nach Anspruch 1, bei denen die überwiegend isotaktischen Propylenpolymere im wesentlichen bestehen aus
(a) 50-100 Gew.-% Propylenpolymeren, hergestellt unter Anwendung von Ziegler-Natta-Katalysatoren oder Metallocenkatalysatoren, vorzugsweise Propylenhomopolymere und/oder Copolymere von Propylen, Ethylen und/oder α-Olefinen mit 4 bis 18 Kohlenstoffatomen und einem Propylenanteil von 80,0 bis 99,9 Gew.-% in Form von statistischen Copolymeren, Blockcopolymeren und/oder statistischen Blockcopolymeren, mit Schmelzindizes von 0,5 bis 40 g/10 min bei 230°C/2,16 kg,
(b) 0-50 Gew.-% einer Polyolefinmischung mit einem Mw/Mn-Verhältnis von 2 bis 6 und einem Schmelzindex von 0,5 bis 40 g/10 min bei 230°C/2,16 kg, im wesentlichen bestehend aus
(b1) 60 bis 98 Gew.-% eines kristallinen Copolymers aus 85 bis 95 Gew.-% Propylen und 15 bis 0,5 Gew.-% Ethylen und/oder eines α-Olefins der allgemeinen Formel CH₂ = CHR, wobei R eine lineare oder verzweigte Alkylgruppe mit 2 bis 8 Kohlenstoffatomen bedeutet,
(b2) 2 bis 40 Gew.-% eines elastischen Copolymers aus 20 bis 70 Gew.-% Ethylen und 80 bis 30 Gew.-% Propylen und/oder eines α-Olefins der allgemeinen Formel CH₂CHR, wobei R eine lineare oder verzweigte Alkylgruppe mit 2 bis 8 Kohlenstoffatomen bedeutet,
(c) 0-30 Gew.-% hochamorpher Polypropylene oder Propylencopolymere mit einem Anteil an kristallinem Polypropylen oder kristallinem Propylencopolymer von weniger als 10 Gew.-%, einer Schmelzenthalpie von weniger als 40 J/g und einem Schmelzindex von 0,5 bis 40 g/10 min bei 230°C/2,16 kg, wobei es sich bei dem weitgehend amorphen Polypropylen um ein Homopolymer des Propylens und/oder ein Copolymer des Propylens aus mindestens 80 Molprozent Propylen und höchstens 20 Molprozent mindestens eines α-Olefins der allgemeinen Formel CH₂CHR, wobei R eine lineare oder verzweigte Alkylgruppe mit 2 bis 8 Kohlenstoffatomen bedeutet, handelt,
(d) 0-10 Gew.-% nichtisotaktischer Propylenhomopolymere mit einem Schmelzpunkt von 145° bis 165°C, einer Schmelzviskosität von 200 Pa.s (200 000 cps) bei 190°C und einer Kristallisationswärme von 4 bis 10 Kalorien pro Gramm sowie einem in Diethylether löslichen Anteil von 35 bis 55 Gew.-%,
(e) 0-30 Gew.-% modifizierter Propylenhomopolymere und/oder Propylencopolymere mit Schmelzindizes von 0,5 bis 40 g/10 min bei 230°C/2,16 kg und einem Quotienten aus der Grenzviskosität des modifizierten Propylenpolymers und der Grenzviskosität des nichtmodifizierten Ausgangspolymers (Komponente a) mit weitgehend gleichem gewichtsmittleren Molekulargewicht von 0,2 bis 0,95.

3. Nichtnachverstreckte Polyolefinfasern nach Anspruch 1 oder 2, bei denen zusätzlich herkömmliche Additive enthalten sind.

4. Nichtnachverstreckte Polyolefinfasern nach Anspruch 3, bei denen als herkömmliche Additive 0,01 bis 2,5 Gew.-% an Stabilisatoren, 0,01 bis 1 Gew.-% an Verarbeitungshilfsmitteln und gegebenenfalls 0,1 bis 1 Gew.-% an Antistatika, 0,2 bis 3 Gew.-% an Pigmenten und 2 bis 20 Gew.-% an Flammschutzmitteln enthalten sind, wobei sich die Prozentangaben jeweils auf die Summe der Polypropylene beziehen.

5. Nichtnachverstreckte Polyolefinfasern nach einem der Ansprüche 1 bis 4, **dadurch gekennzeichnet, daß** in den überwiegend isotaktischen Propylenpolymeren 5-100 ppm an Teilchen anorganischer Oxide mit einem Teilchendurchmesser von 0,05-10 µm enthalten sind.

6. Nichtnachverstreckte Polyolefinfasern nach Anspruch 5, **dadurch gekennzeichnet, daß** in den überwiegend isotaktischen Propylenpolymeren 20-40 ppm an anorganischen Teilchen aus der Gruppe ZnO, SnO, MgO, Al₂O₃, SiO₂, TiO₂, ZrO₂, HfO₂ und deren Mischungen enthalten sind.

7. Nichtnachverstreckte Polyolefinfasern nach einem der Ansprüche 5 oder 6, **dadurch gekennzeichnet, daß** die Teilchen aus anorganischen Oxiden Al₂O₃ und/oder SiO₂ und/oder MgO mit einem Teilchendurchmesser von 0,5 bis 2,0 µm sind.

8. Verfahren zur Herstellung nichtnachverstreckter Polyolefinfasern gemäß einem der Ansprüche 1 bis 7, **dadurch gekennzeichnet, daß** man überwiegend isotaktische Propylenpolymere gemäß einem der Ansprüche 1 bis 7 und 0,001 bis 2 Gew.-% bezogen auf die eingesetzten Propylenpolymere, an α-Nukleierungsmitteln gemäß Anspruch 1 bei Temperaturen von 220 bis 325°C aufschmilzt, die Schmelze Spinndüsen zuführt, die Schmelze zu Fasern ausformt und anschließend die Fasern kühlt und mit Geschwindigkeiten von 1000 - 6000 m/min aufnimmt.

9. Verfahren zur Herstellung nichtnachverstreckter Polyolefinfasern nach Anspruch 8, **dadurch gekennzeichnet, daß** man mit schnellaufenden Galetten aufnimmt, die Fasern zu multifilen Garnen zusammenführt und die die nicht nachverstreckten Polyolefinfasern enthaltenden Garne aufwickelt.

10. Verwendung nichtnachverstreckter Polyolefinfasern gemäß einem der Ansprüche 1 bis 7 zur Herstellung von Vliesstoffen, für textile Anwendungen sowie Teppiche.

11. Nichtnachverstreckte Polyolefinfasern nach Anspruch 2, bei denen die Propylenpolymere gemäß 2 (a) Schmelzindizes von 1 bis 5 g/10 min bei 230°C/2,16 kg aufweisen.

12. Nichtnachverstreckte Polyolefinfasern nach Anspruch 2, bei denen die modifizierten Propylenhomopolymere und/oder Propylencopolymere gemäß 2 (e) Schmelzindizes von 2 bis 5 g/10 min bei 230°C/2,16 kg aufweisen.

13. Verwendung nichtnachverstreckter Polyolefinfasern nach Anspruch 10, **dadurch gekennzeichnet, daß** es sich bei den Vliesstoffen um Spinnvliese, kardierte oder durch Airbonding verbundene Vliesstoffe handelt.

## Revendications

1. Fibres de polyoléfine non étirées postérieurement ayant des valeurs de ténacité élevées de 2,0 à 5,0 cN/dtex, essentiellement constituées de polymères de propylène majoritairement isotactiques ayant une température de cristallisation de > 116°C (DSC) et de 0,001 à 2% en poids, par rapport aux polymères de propylène employés, d'agents de nucléation en α qui sont choisis dans le groupe constitué par
les polymères qui sont différents des polymères de propylène isotactiques, qui sont choisis dans le groupe constitué par
les polymères de tétrafluoroéthylène, les polycarbonates, le poly(butylène-téréphtalate), le poly-(éthylène-téréphtalate), les polymères de 3-méthylbutène, les polymères de 4-méthylpentène-1, les polymères de propylène syndiotactiques, les poly(oxydes de phénylène), les copolymères propylène-méthylbutène, les copolymères styrène-acrylonitrile, les polyallyltriméthylsilanes et les copolymères éthylène-acétate de vinyle hydrolysés,
et l'acide benzoïque, les dérivés d'acide benzoïque, le dibenzylidènesorbitol, les dérivés de sorbitol, la diphénylglycine, les sels d'acides carboxyliques aliphatiques en C₆-C₁₈, les sels d'acides carboxyliques aromatiques en C₇-C₁₃, les dérivés d'acide phosphorique, le talc et leurs mélanges.

2. Fibres de polyoléfine non étirées postérieurement selon la revendication 1, dans lesquelles lesdits polymères de propylène majoritairement isotactiques sont essentiellement constitués par
(a) 50 - 100% en poids de polymères de propylène produits au moyen de catalyseurs de Ziegler-Natta ou de catalyseurs métallocène, de préférence d'homopolymères de propylène et/ou de copolymères de propylène, d'éthylène et/ou d'α-oléfines comportant 4 à 18 atomes de carbone et ayant une teneur en propylène de 80,0 à 99,9% en poids sous forme de copolymères statistiques, de copolymères séquencés et/ou de copolymères séquencés statistiques, ayant des indices de fluidité à chaud de 0,5 à 40 g/10 min à 230°C/2,16 kg,
(b) 0 - 50% en poids d'un mélange de polyoléfines présentant un rapport Mp/Mn ratio de 2 à 6 et ayant un indice de fluidité à chaud de 0,5 à 40 g/10 min à 230°C/2,16 kg, essentiellement constitué de
(b1) 60 à 98% en poids d'un copolymère cristallin de 85 à 95% en poids de propylène et de 15 à 0,5% en poids d'éthylène et/ou d'une α-oléfine de formule générale CH₂ = CHR, dans laquelle R est un groupe alkyle linéaire ou ramifié de 2 à 8 atomes de carbone,
(b2) 2 à 40% en poids d'un copolymère élastique de 20 à 70% en poids d'éthylène et de 80 à 30% en poids de propylène et/ou d'une α-oléfine de formule générale CH₂CHR, dans laquelle R est un groupe alkyle linéaire ou ramifié de 2 à 8 atomes de carbone,
(c) 0 - 30% en poids de polypropylènes ou de copolymères de propylène hautement amorphes ayant une teneur en polypropylène cristallin ou en copolymère de propylène cristallin inférieure à 10% en poids, une enthalpie de fusion inférieure à 40 J/g et un indice de fluidité à chaud de 0,5 à 40 g/10 min à 230°C/2,16 kg, le polypropylène essentiellement amorphe étant un homopolymère de propylène et/ou un copolymère de propylène d'au moins 80 pour cent en moles de propylène et de pas plus de 20 pour cent en moles d'une ou plusieurs α-oléfines de formule générale CH₂CHR, dans laquelle R est un groupe alkyle linéaire ou ramifié de 2 à 8 atomes de carbone,
(d) 0 - 10% en poids d'homopolymères de propylène non isotactiques ayant un point de fusion de 145° à 165°C, une viscosité à chaud de 200 Pa.s (200 000 cP) à 190°C et une chaleur de cristallisation de 4 à 10 calories par gramme, 35 à 55% en poids étant soluble dans l'éther diéthylique,
(e) 0 - 30% en poids d'homopolymères de propylène et/ou de copolymères de propylène modifiés ayant des indices de fluidité à chaud de 0,5 à 40 g/10 min à 230°C/2,16 kg, et un rapport entre la viscosité intrinsèque du polymère de propylène modifié et la viscosité intrinsèque du polymère non modifié de base (constituant a) ayant essentiellement la même masse moléculaire moyenne en poids de 0,2 à 0,95.

3. Fibres de polyoléfine non étirées postérieurement selon la revendication 1 ou 2, comprenant en outre des additifs classiques.

4. Fibres de polyoléfine non étirées postérieurement selon la revendication 3, dans lesquelles lesdits additifs classiques sont 0,01 à 2,5% en poids de stabilisants, 0,01 à 1% en poids d'adjuvants de traitement et, le cas échéant, 0,1 à 1% en poids d'agents antistatiques, 0,2 à 3% en poids de pigments et 2 à 20% en poids d'ignifugeants, dans chaque cas par rapport à la somme des polypropylènes.

5. Fibres de polyoléfine non étirées postérieurement selon l'une quelconque des revendications 1 à 4 **caractérisées en ce que** les polymères de propylène majoritairement isotactiques comprennent de 5 à 100 ppm de particules d'oxydes minéraux ayant un diamètre de particule de 0,05 - 10 *µ*m.

6. Fibres de polyoléfine non étirées postérieurement selon la revendication 5, **caractérisées en ce que** les polymères de propylène majoritairement isotactiques comprennent de 20 à 40 ppm de particules minérales choisies dans le groupe constitué par ZnO, SnO, MgO, Al₂O₃, SiO₂, TiO₂, ZrO₂, HfO₂ et leurs mélanges.

7. Fibres de polyoléfine non étirées postérieurement selon une des revendications 5 ou 6, **caractérisées en ce que** les particules d'oxydes minéraux sont Al₂O₃ et/ou SiO₂ et/ou MgO ayant un diamètre de particule de 0,5 à 2,0 *µ*m.

8. Procédé de préparation de fibres de polyoléfine non étirées postérieurement selon l'une quelconque des revendications 1 à 7, **caractérisé par** la fusion de polymères de propylène majoritairement isotactiques selon l'une quelconque des revendications 1 - 7 et de 0,001 à 2% en poids, par rapport aux polymères de propylène employés, d'agents de nucléation en α selon la revendication 1 à des températures de 220 à 325°C, le transport de la masse fondue vers des filières, l'extrusion de la masse fondue en fibres, puis le refroidissement des fibres et le bobinage des fibres filées à chaud à des vitesses de 1000 - 6000 m/min.

9. Procédé de préparation de fibres de polyoléfine non étirées postérieurement selon la revendication 8, **caractérisé en ce que** la fibre filée à chaud est bobinée par des galettes à grande vitesse, les fibres sont câblés en fils multifilaments et les fils contenant les fibres de polyoléfine non étirées postérieurement sont bobinées.

10. Utilisation de fibres de polyoléfine non étirées postérieurement selon l'une quelconque des revendications 1 à 7 pour fabriquer des non-tissés, pour des applications textiles, et des tapis.

11. Fibres de polyoléfine non étirées postérieurement selon la revendication 2, dans lesquelles les polymères de propylène selon 2 (a) ont des indices de fluidité à chaud de 1 à 5 g/10 min à 230°C/2,16 kg.

12. Fibres de polyoléfine non étirées postérieurement selon la revendication 2, dans lesquelles les homopolymères de propylène et/ou les copolymères de propylène modifiés selon 2 (e) ont des indices de fluidité à chaud de 2 à 5 g/10 min à 230°C/2,16 kg.

13. Utilisation de fibres de polyoléfine non étirées postérieurement selon la revendication 10, **caractérisées en ce que** les non-tissés sont des non-tissés filés-liés, cardés ou par voie sèche aérodynamique.
